

# UNITED STATES PATENT OFFICE.

DOUGLAS E. SCOTT, OF BOSTON, MASSACHUSETTS, ASSIGNOR TO ARTHUR D. LITTLE, INCORPORATED, OF CAMBRIDGE, MASSACHUSETTS, A CORPORATION OF MASSACHUSETTS.

## PROCESS OF ISOLATING FIBER FROM BAGASSE.

1,399,891.

Specification of Letters Patent.

Patented Dec. 13, 1921.

No Drawing.

Application filed August 7, 1918. Serial No. 248,809.

To all whom it may concern:

- Be it known that I, DOUGLAS E. SCOTT, a citizen of the United States, residing at Boston, Roxbury district, in the county of 5 Suffolk and State of Massachusetts, have invented certain new and useful Improvements in Processes of Isolating Fiber from Bagasse, of which the following is a specification.
- 10 This invention is a process of treating bagasse (the residue from the crushing of sugar cane) for the purpose of preparing therefrom a clean fiber suitable for paper-making or other purposes.
- 15 Efforts have long been made, with varying degrees of success, to isolate from bagasse a fiber which should conform in all respects to the requirements of the paper maker. According to the present invention 20 this is accomplished in a cheap and expeditious manner, and in course of a single operation which effects the disintegration of the bagasse and the detachment of the pith from the fiber, the elimination of those pithy 25 components which are undesirable in paper stock, and the removal of the large quantity of dirt and insoluble matter which always accompanies bagasse by reason of the conditions under which sugar cane is harvested.
- 30 According to the present invention, the bagasse in the form in which it is usually delivered by the sugar mill to the burners, is preferably but not necessarily subjected to a supplemental shredding, or shredding 35 and crushing, operation. The purpose of this treatment, for which any of the standard shredding devices may be used, is primarily to shorten the time required for the subsequent operation; and the desirability 40 of the supplemental shredding would of course depend somewhat upon the physical condition, including the state of subdivision of the bagasse itself; for, as is well understood in this art, the physical condition of 45 bagasse from different mills varies rather widely according to the intensity and number of the crushing, or shredding and crushing, operations to which it has been subjected.
- 50 Whether shredded or not, the bagasse in the moist condition is charged into an apparatus designed and adapted to disintegrate further and minutely the material into its structural elements and to do this in the presence of a relatively large proportion of 55 water, which may well be twenty-five to fifty times the weight of the bagasse. The apparatus must be equipped with a suitable screening device adapted to wet screening and provided with screen of a mesh relatively very coarse as compared with the screens or wires heretofore used in paper-making. The essential point relative to the choice of this mesh is that it should be capable of effecting a reasonably perfect separation as between the pith and fiber, after 60 which the latter is in proper condition for the ensuing cooking operation. The ordinary paper mill beater, equipped with a washer, may be adapted to the purposes of 65 the process, the usual fine mesh wire of the washing cylinder being replaced, however, by the relatively coarse mesh above mentioned.
- 70 The operation of separating the pith from the fiber is to be distinguished clearly from the common practice of washing the fiber in the beater. The latter operation is performed upon cooked fiber and has for its primary purpose the removal of soluble 75 matters. Hence the screen used is always of close mesh (usually about #70) in order to retain all vegetable structures and plant 80 cells. In the present case, on the contrary, the treatment in the beater or equivalent devices precedes the cooking operation, and is 85 so conducted as to accomplish a progressive breaking down or disintegration of the plant structure with coincident screening out and removal of the pith component. Consequently the size of the screen mesh must for 90 the purpose of this process be of such order and dimensions as to permit passage of pith cells while preventing passage of fiber and fiber bundles. For this purpose a screen 95 about #12 mesh is satisfactory.
- 95 The beating operation is more or less prolonged according to the physical state of the bagasse at the time of its introduction into the beater. In the case of bagasse which 100 has been subjected to a supplemental shredding and crushing, treatment in the beater for about one hour will usually suffice to accomplish the desired results, comprising in addition to the washing out of the residual sugar content:
- (1) Detaching the particles of pith from the fibrous stock, and so far disintegrating

the latter as to bring it into the best condition for the subsequent cooking operation;

(2) Washing the pithy particles out through the washing cylinder, and thereby 5 eliminating them so far as the paper-making operation is concerned. This phase of the treatment bears considerable resemblance to the washing of rag stock, except that in the latter case most of the material which is 10 eliminated passes off in solution.

(3) Eliminating a large amount of dirt and insoluble matter which could not be removed in course of any of the subsequent processes of paper-making. For example 15 much of this dirt would fail to subside through the mass of stock in such way as to be caught by the sand-catcher of the beater; nor would it be caught by the screen of a paper machine. The rotary cylinder 20 washer covered with a relatively coarse screen as above described has proven highly

effective both in the elimination of the pith and in the washing of the fiber.

The purified and washed fiber prepared as above is now ready for the cooking operation and for the subsequent manipulations by which it is converted into paper of the desired quality. 25

I claim:—

1. Process of isolating fiber from bagasse, 30 which consists in subjecting the raw material in the presence of water to mechanical forces causing progressive disintegration of the material and detachment of the pith from the fiber and simultaneously removing 35 the insoluble impurities and the pith by screening while retaining the purified fiber.

2. Process according to claim 1 in which the raw material is preliminarily shredded.

In testimony whereof I affix my signature. 40

DOUGLAS E. SCOTT.